# EUROPEAN PATENT SPECIFICATION

(11) **EP 0 229 172 B1**
(45) Date of publication and mention of the grant of the patent: **06.05.1992**
(21) Application number: 86904673.0
(22) Date of filing: 08.07.1986
(51) Int. Cl.: D01F 8/00

(54) **SHEATH CORE FIBER AND ITS METHOD OF MANUFACTURE**
FASER MIT KERN UND UMHÜLLUNG UND DEREN HERSTELLUNG
FIBRES A NOYAU ET A GAINE ET SON PROCEDE DE PRODUCTION

(30) Priority: 12.07.1985 US 754327
(43) Date of publication of application: 22.07.1987
(73) Proprietor: OHIO UNIVERSITY, Athens, OH 45701 (US)
(72) Inventor: COLLIER, John, R., Athens, OH 45701 (US); COLLIER, Billie, J., Athens, OH 45701 (US)
(74) Representative: Baillie, Iain Cameron
(86) International application number: US8601473
(87) International publication number: WO8700561

(56) References cited:
- DE-B- 1 174 291
- GB-A- 764 954

## Description

The present invention relates to sheath core fibers.

The desirability of combining the optimum characteristics oriented thermoplastic materials, such as maintenance of crease and tear resistance, with the dyeability and sorptivity of natural materials has been recognized for some time. Attempts in this direction have usually resulted in blending the two materials together so that there is an averaging of the properties of the material rather than an optimization of each of the component's most desirable properties.

Coextrusion of two different materials to form a side-by-side bicomponent fiber has been done extensively, primarily to develop a crimped product. For example, U.S. Patent No. 2,439,813, Kulp, discloses such a product, where both components are viscose of different contractivity due to different aging times and different concentrations of cellulose, carbon disulfide, or sodium hydroxide. Sheath core structures have also been formed, again usually for crimping purposes. For example, U.S. Patent No. 3,458,615, Bragaw, discloses a coextrusion of two streams in the molten state and any orientation to be developed will be induced downstream from the die. The Bragaw patent is directed to the production of light guides where a well controlled smooth interface is critical to maintaining internal reflection of the light passing through the core and reflected off the surface. U.S. Patent No. 2,932,079, Dietzsch, discloses a sheath core structure which must contain at least two cores of different materials and a sheath of a third material. This is so that crimp may be developed by differential thermal contraction of non-concentric core and sheath layers. U.S. Patent No. 2,989,798, Bannerman, is also involved in the production of a sheath core fiber in which both layers are polyamides. The core polyamide is chosen or modified to be more dye receptive. U.S. Patent No. 2,063,180, Meyer, involves a coextrusion process in which an inner stream consisting of a volatile solvent carrying a coloring substance passes through a wick and is subsequently covered by a viscose solution. During spinning the volatile solvent diffuses through the forming rayon leaving behind only the coloring substance. The inner core would not exist as a discrete region since the dye would form a gradient into the rayon.

U.K. Patent 764,954 is concerned with the problem of dying or printing fibrous material of thermoplastic synthetic resin. The patent teaches applying to the fibrous material a solution yielding regenerated cellulose protein or polyvinyl alcohol on precipitation. It is indicated that the coating obtained will impart dye stuff affinity. The citation is concerned with "fibrous material" which may be in the form of "staple fiber material yarns, threads, fabrics or knitted goods". All of the examples are concerned with the treatment of fabrics.

U.S. Patent 2,312,469 discloses a formulation for a protein size to be applied to nylon yarns to aid in subsequent processing into knitted goods. The objective is simply to protect the yarns during knitting and subsequent handling and the coating binds the fibers together in a coherent structure for knitting. The coating is then removed and thus is not an integral part of the structure of each fiber of the yarn.

U.S. Patent No. 4,382,111 discloses the treatment of fibers, as well as yarns. However, all of the examples of the treatment of fibers are when they are in the yarn state. Furthermore, the subliminal substance to which the yarns are exposed is to be used as a lubricant and is removable by sublimation without the application of additional procedures after the formation of the fiber products and is not during ultimate usage adherent to the individual fibers.

Similarly, DE-B-1174291 is concerned with the treatment of yarns and textile materials and does not provide an individual fiber having thereon a continuous sheath.

In accordance with this invention, there is provided a sheath core fiber comprising an inner continuous core of an oriented thermoplastic material coated with an adherent organic polymeric sheath made of a non- thermoplastic material, and excluding sheath core fibers wherein the sheath is readily removable from said core and is not retained on said core during ultimate usage of said fiber, characterized by said sheath being continuous along the length of the fiber and completely surrounding it, and said sheath having microscopic surface dimpling of a type indicative of a lack of orientation of the surface of the sheath.

In accordance with another aspect of the invention, there is provided a method of making a sheath core fiber comprising an inner continuous core of an oriented thermoplastic material coated with an adherent organic polymeric sheath made of a nonthermoplastic material, characterized by drawing the core through the sheath forming material in liquid form, thence drawing said core through a die so that the desired thickness of sheath forming material remains on said core, drawing said thus coated core through an acid bath to coagulate the sheath material on said core, and rinsing said resulting sheath core fiber with water.

Because the core fiber is already oriented and in solid form, there is a very low tensile load on the sheath material and thus it will not develop significant crystal orientation during the drawing process, as would be the case if it alone were being drawn from the die. This results in the production of a sheath material which is not oriented and, consequently, has increased sorptivity and dyeability. Yet, because the core material constitutes the major cross section of the fiber, it will maintain the strength and crease and tear resistance which are characteristic of the core material. In producing this fiber, because of the tensile strength of the existing inner core structure, it is not necessary to coagulate the sheath material immediately as it exits from the die. Thus the die face does not have to be in contact with the acid bath as is the case of a viscose fiber being drawn from a die. This lessens the necessity of having the die face constructed of precious metal and significantly simplifies and reduces the cost of manufacturing the product.

It is therefore an object of this invention to provide a sheath core fiber combining the most desirable characteristics of the core, coupled with the most desirable characteristics of the sheath.

It is also an object of this invention to provide a method of making such a product.

These, together with other objects and advantages of the invention, will become apparent from the following detailed description of the invention.

Fig. 1 is a schematic diagram of the method of producing the fiber of this invention.

Fig. 2 is a perspective view of a single fiber.

Fig. 3 is a scanning electron micrograph of a fiber produced by this invention at a magnification of 1250x.

Referring now to the drawings, and particularly to Fig. 1, in the method of making the fiber of this invention, the core material 10 is introduced into the chamber 11, which is provided with a die 12 at its lower end. The liquid sheath-forming material is introduced through member 13 by gravity or pressure flow into the chamber 11. The fiber solution contact region is designed to be sufficient to insure that the core 10 is thoroughly coated with the sheath-forming material prior to entering the die 12. The relative amount of solution coated onto the core fiber is controlled by die opening geometry, solution rheological properties, and drag and pressure driven flow. The combined sheath core fiber 14 exits the die 12 and enters the acid bath 15 where the sheath material is coagulated. The sheath core fiber 14 exits the acid bath 15, is rinsed with a water rinse 16, and is then collected on take-up roll 17.

Referring now more particularly to Fig. 2, the core material 10 is shown with the sheath material 18 surrounding the core material. Satisfactory fibers where the core 10 is 20 µm in diameter and the sheath material 18 is one µm in thickness have been produced. Thicker sheath layers have also been produced by increasing the pressure imposed in member 13.

Fig. 3, which is a scanning electron micrograph of the sheath core fiber shown in Fig. 2 at a magnification of 1250x, reveals dimples that are not elongated indicating lack of orientation of the surface and the enhanced surface area. Both of these properties contribute high sorptivity and thus comfort and dyeability. The method of producing such a fiber is described in detail in the following example which involves nylon 66 for the core and viscose rayon for the sheath. While the invention is described with respect to these two materials, and this is a preferred combination, it must be kept in mind that other core materials and other sheath materials are contemplated within the scope of this invention.

### EXAMPLE 1

An already oriented nylon fiber was passed through a commercial viscose rayon solution and then drawn through a die. The core fiber was nylon 66 and was 20 µm in diameter. The die opening was approximately 800 µm and the resultant rayon skin thickness was one µm. The line speed of 30.5m (100 feet) per minute was used with a commercial concentration spinning bath consisting of nine weight percent sulfuric acid and 13 weight percent of sodium sulfate. Much higher line speeds, of course, can be used and different die openings and/or a higher pressure head may also be used. The resulting fibers maintain essentially the bulk mechanical properties of the nylon core and have the dyeability of rayon.

Commercial rayon fibers typically are formed from a solution containing about seven percent cellulose in a sodium xanthate form and seven percent alkali. An acceptable viscosity for spinning is achieved by ripening the viscose solution for four to five days. The fibers are formed by extruding thin filaments of this solution from a spinning bath in which the cellulose is regenerated from its xanthate form and coagulated. This is performed under tension and orientation develops in the rayon fiber, the level of which is controlled by the tension, cellulose source and character, and the spinning bath concentration and temperature.

In the instant invention, since the core material carries the tensile load, the sheath material develops very low, if any, orientation, as opposed to normal rayon fibers that are spun under tension to develop strength relating to orientation. This enables surface dimpling which results in an enhanced surface area contributing to higher sorptivity and greater dyeability. Furthermore, since the core material carries the tensile load, the acid bath, as shown in Fig. 1, can be spaced from the face of the die and thus precious metal faced dies are not needed in practicing this invention. In addition, since this process does not require the viscose solution to be able to be drawn into a fiber, a broader class of viscose solutions may be used.

While this invention has been described in its preferred embodiment, it is appreciated that slight variations may be made without departing from the scope of the invention.

## Claims

1. A sheath core fiber comprising an inner continuous core (10) of an oriented thermoplastic material coated with an adherent organic polymeric sheath (18) made of a nonthermoplastic material, and excluding sheath core fibers wherein the sheath is readily removable from said core and is not retained on said core during ultimate usage of said fiber, characterized by said sheath being continuous along the length of the fiber and completely surrounding it, and said sheath having microscopic surface dimpling of a type indicative of a lack of orientation of the surface of the sheath.

2. A sheath core fiber according to claim 1, characterized by the fact that the thermoplastic material is selected from the group consisting of nylons, polyesters, acrylics and olefins and the organic polymeric sheath comprises a material selected from the group consisting of regenerated cellulose, and regenerated protein.

3. A sheath core fiber according to claim 1 characterized by said sheath (18) having a desired uniform thickness as a consequence of the use of a fabricating process in which a single fiber core, coated with a polymer sheath forming material in liquid form, is drawn through a die.

4. A method of making a sheath core fiber comprising an inner continuous core (10) of an oriented thermoplastic material coated with an adherent organic polymeric sheath (18) made of a nonthermoplastic material, characterized by drawing the core through the sheath forming material in liquid form, thence drawing said core through a die so that the desired thickness of sheath forming material remains on said core, drawing said thus coated core through an acid bath to coagulate the sheath material on said core, and rinsing said resulting sheath core fiber with water.

5. A method according to claim 4, characterized by the fact that the core is made of a material selected from the group consisting of polyesters, nylons, acrylics, and olefins.

6. A method according to claims 4 or 5, characterized by the fact that the sheath forming material is selected from the group consisting of regenerated cellulose and regenerated protein.

## Revendications

1. Fibre à noyau et à gaine comprenant un noyau interne continu (10) en matière thermoplastique orientée revêtu d'une gaine polymérique organique adhérente (18) en matière non thermoplastique, à l'exclusion des fibres à noyau et à gaine dans lesquelles la gaine est facile à séparer dudit noyau et n'est pas maintenue sur ledit noyau pendant l'utilisation ultime de ladite fibre, caractérisée en ce que ladite gaine est continue sur la longueur de la fibre et l'entoure totalement, et en ce que ladite gaine présente un ondulation superficielle microscopique d'un type qui indique une absence d'orientation de la surface de la gaine.

2. Fibre à noyau et à gaine selon la revendication 1, caractérisée par le fait que la matière thermoplastique est choisie dans le groupe formé par les Nylon, les polyesters, les acryliques et les oléfines et la gaine polymérique organique comprend une matière choisie dans le groupe formé par la cellulose régénérée et les protéines régénérées.

3. Fibre à noyau et à gaine selon la revendication 1, caractérisée en ce que ladite gaine (18) présente une épaisseur uniforme souhaitée par suite de l'utilisation d'un procédé de fabrication dans lequel on fait passer dans une filière un noyau de fibre unique, revêtu d'une matière formant gaine polymérique sous forme liquide.

4. Procédé de fabrication d'une fibre à noyau et à gaine comprenant un noyau interne continu (10) en matière thermoplastique orientée revêtu d'une gaine polymérique organique adhérente (18) en une matière non thermoplastique, caractérisé en ce qu'on fait passer le noyau dans la matière formant gaine sous forme liquide, puis dans une filière de sorte que l'épaisseur souhaitée de matière formant gaine reste sur ledit noyau, on fait passer ledit noyau ainsi revêtu dans un bain d'acide pour coaguler la matière formant gaine sur ledit noyau et on rince à l'eau ladite fibre à noyau et à gaine obtenue.

5. Procédé selon la revendication 4, caractérisé par le fait que le noyau est constitué par une matière choisie dans le groupe formé par les polyesters, les Nylon, les acryliques et les oléfines.

6. Procédé selon les revendications 4 ou 5, caractérisé par le fait que la matière formant gaine est choisie dans le groupe formé par la cellulose régénérée et les protéines régénérées.

## Patentansprüche

1. Kernmantelfaser, umfassend einen inneren durchgehenden Kern (10) aus einem gerichteten thermoplastischen Material, welches mit einem haftenden Mantel (18) auf der Basis eines organischen Polymers aus einem nichtthermoplastischen Material überzogen ist, und ausgenommen Kernmantelfasern, bei denen der Mantel leicht von dem Kern abzulösen ist und während des endgültigen Gebrauchs der Faser nicht auf dem Kern bleibt, dadurch gekennzeichnet, daß der Mantel auf der Länge der Faser durchgehend ist und sie vollständig umgibt, und daß der Mantel auf seiner Oberfläche mikroskopisch kleine Vertiefungen aufweist, die auf eine mangelnde Ausrichtung der Oberfläche des Mantels hindeuten.

2. Kernmantelfaser nach Anspruch 1, dadurch gekennzeichnet, daß das thermoplastische Material ausgewählt ist aus der Gruppe umfassend Nylon, Polyester, Acryl und Olefine, und daß der Mantel aus organischem Polymer ein Material enthält, das ausgewählt ist aus der Gruppe umfassend regenerierte Cellulose und regeneriertes Protein.

3. Kernmantelfaser nach Anspruch 1, dadurch gekennzeichnet, daß der Mantel (18) eine gewünschte gleichmäßige Dicke aufweist aufgrund der Verwendung eines Herstellungsverfahrens, bei dem ein Einzelfaserkern, der mit einem Polymermantel überzogen ist, welcher ein Material in flüssiger Form darstellt, durch eine Ziehdüse gezogen wird.

4. Verfahren zur Herstellung einer Kernmantelfaser mit einem inneren durchgehenden Kern (10) aus einem gerichteten thermoplastischen Material, welches mit einem haftenden Mantel (18) auf der Basis eines organischen Polymers aus einem nichtthermoplastischen Material überzogen ist, gekennzeichnet durch die folgenden Schritte: Ziehen des Kerns durch das mantelbildende Material in flüssiger Form, dann Ziehen des Kerns durch eine Ziehdüse, so daß das mantelbildende Material in der gewünschten Dicke auf dem Kern bleibt, Ziehen des so überzogenen Kerns durch ein Säurebad, um das Mantelmaterial auf dem Kern zu koagulieren, und Spülen der entstehenden Kernmantelfaser mit Wasser.

5. Verfahren nach Anspruch 4, dadurch gekennzeichnet, daß der Kern aus einem Material besteht, welches ausgewählt ist aus der Gruppe umfassend Polyester, Nylon, Acryl und Olefine.

6. Verfahren nach Anspruch 4 oder 5, dadurch gekennzeichnet, daß das mantelbildende Material ausgewählt ist aus der Gruppe umfassend regenerierte Cellulose und regeneriertes Protein.
